

# UNITED STATES PATENT OFFICE.

CHARLES FREDERICK CROSS AND JOHN FREDERICK BRIGGS, OF LONDON, ENGLAND.

## PROCESS OF MAKING A CELLULOSE MATERIAL.

No. 920,828.

Specification of Letters Patent.

Patented May 4, 1909.

Application filed September 16, 1907. Serial No. 393,190. (Specimens.)

*To all whom it may concern:*

Be it known that we, CHARLES FREDERICK CROSS and JOHN FREDERICK BRIGGS, subjects of the King of Great Britain, residing at 3 and 4 New Court, Lincolns Inn, in the county of London, England, chemists, have invented a certain new and useful Process of Making a Cellulose Material, of which the following is a specification.

10 The properties of cellulose are considerably changed by introducing into the compound various acid radicals; for instance by introducing organic acid radicals, notably the acetyl group, into cellulose, the behavior 15 of the product varies from that of cellulose in many respects. Thus acidulated, particularly acetylated, cellulose exhibits as is known more or less resistance to direct cotton dyestuffs; it is less subject to the action 20 of alkalies, as in the mercerizing process, and has a diminished attraction for atmospheric moisture. The advantages which can readily be foreseen as likely to accrue from such alteration in the properties of this 25 textile material have never been realized, however, for the reason that such processes as have been devised for introducing the radicals or groups in question so attack the fibrous cellulose that it does not retain sufficient 30 of its original structure and strength to be suitable for spinning or weaving. As an example, the acetylated processes hitherto described have yielded as final products higher acetylated celluloses. These higher 35 esters are soluble in chloroform, nitrobenzene, acetic acid, and other organic liquids, which property is an essential condition of their technical applications.

40 The properties of cellulose are considerably changed by introducing into the compound various acid radicals; for instance by introducing organic acid radicals, notably the acetyl group, into cellulose, the behavior 45 of the product varies from that of cellulose in many respects. Thus acidulated, particularly acetylated cellulose exhibits as is known more or less resistance to direct cotton dyestuffs; it is less subject to the action of alkalies, as in the mercerizing process, and 50 has a diminished attraction for atmospheric moisture. The advantages which can readily be foreseen as likely to accrue from such alteration in the properties of this textile material have, however, never been realized, 55 for the reason that such processes as have

been devised for introducing the radicals or groups in question so attack the fibrous cellulose that it does not retain sufficient of its original structure and strength to be suitable for spinning or weaving. As an example, the 60 acetylated processes hitherto described have yielded as final products higher acetylated celluloses. These higher esters are soluble in organic liquids, which property is an essential condition of their technical applications. 65 In the numerous inventions of recent years for preparing the higher acetic esters of cellulose, the reaction is preceded by hydrolysis of the cellulose, and this stage is recognized as determined by an auxiliary reagent, speci- 70 fied as an essential component of the acety- lating mixture. One of these methods is de- scribed as consisting in simultaneously hy- drolyzing and acetyating the cellulose by treatment with acetic anhydrid and sulfuric 75 acid or primary salts thereof or other mineral acids. This condition of acid attack im- ports the disintegration of the cellulose fibers more or less and hence excludes its applica- 80 tion to cellulose yarns or fabrics, or to fibers to be afterward employed in textile manu- factures. It has nevertheless been proposed to treat textile fabrics with such acetyating mixtures, to produce a partial, in the sense of superficial, conversion of the cellulose into 85 acetate. No indications are given for con- trolling the process in its industrial applica- 90 tion.

The process according to the present in- vention is by contrast a conversion of the cel- lulose in the mass, free from the dangers of acid disintegration or weakening of the fibers limited definitely to the lower grades of acety- lization, and carried out under conditions 95 which produce regular and definite products with a minimum consumption of reagents.

Our invention consists in a method of treating fibrous cellulose with appropriate known acetyating agents, in such a manner that it is converted into lower acetyl deriva- 100 tives without prejudice to the textile qualities.

Our invention consists in treating fibrous cellulose with appropriate known acetyating agents, in such a manner that it is converted 105 into lower acetyl derivatives without prejud- ice to the textile qualities of the fiber. These lower acetylated products are specific- 110 ally insoluble in the organic solvent liquids mentioned above.

The process is applicable to the fiber itself, to yarn or to woven or otherwise manufactured fabrics, and we thus obtain for the first time cellulose ester derivatives which 5 while retaining the textile quality of the fiber or fabric, resist substantive cotton dyestuffs and can be subjected to alkaline lye in a mercerizing treatment without being sensibly altered.

- 10 We subject the cellulose to the limited acetylation action of acetic anhydrid aided by a suitable saline assisting or condensing agent that has little or no effect on the fiber, such as zinc chlorid. A satisfactory criterion that the desired acetylation has been 15 attained is the increase in weight of the cellulose, which may be from 15 to 50 per cent., according to requirements; the proportion of the mixture of acetic anhydrid and zinc 20 chlorid which the cellulose is allowed to absorb, as well as the extent to which the mixture is to be diluted with say glacial acetic acid or the like, are determined by 25 the required degree of acetylation.
- 25 In carrying out the process we generally adjust the proportion of liquid to cellulose according to the absorption capacity of the raw material, so that the liquid is held uniformly distributed throughout the mass 30 of cellulose. The degree of modification ultimately obtained is then regulated by varying the proportion of the diluting agent in the liquid.

As a specific example, assuming that 35 ton yarn or cotton cloth is to be acetylated so as to have the power of resisting direct cotton dyestuffs or mercerization, the thoroughly dried material is uniformly saturated with the liquid in such a manner 40 that it retains approximately the predetermined quantity. This quantity depends on the degree of modification required and therefore on the percentage gain in weight of the cellulose. For a gain in weight of 45 approximately 25 per cent. the dry cellulose may be caused to absorb twice its weight of a mixture having the following composition.

50

|                      |      |                  |
|----------------------|------|------------------|
| Acetic anhydrid.     | 42   | parts by weight. |
| Acetyl chlorid.      | 11.5 | " "              |
| Glacial acetic acid. | 50   | " "              |
| Ignited zinc oxid.   | 6.5  | " "              |

The zinc oxid and acetyl chlorid are used instead of zinc chlorid, being more convenient on account of the water which inevitably accompanies zinc chlorid; obviously, zinc 55 acetate may be substituted for the zinc oxid.

For a gain in weight of approximately 33 per cent. 1 part of the cellulose may be caused to absorb 2.3 parts of a mixture composed of

60

|                      |      |                  |
|----------------------|------|------------------|
| Acetic anhydrid.     | 56   | parts by weight. |
| Acetyl chlorid.      | 11.5 | " "              |
| Glacial acetic acid. | 32   | " "              |
| Ignited zinc oxid.   | 6.5  | " "              |

In preparing such mixtures the liquid constituents are first mixed together and 65 the zinc oxid is added in small quantities

at a time, the mixture being stirred and cooled if necessary until the whole is dissolved.

When zinc chlorid is used as such, a suitable mixture is prepared by dissolving 20 70 parts of commercial zinc chlorid in 80 parts of glacial acetic acid and adding to the solution 100 parts of acetic anhydrid, these proportions being suitable for obtaining a gain of weight amounting to 20-40 per cent., 75 according to the quantity used.

It is to be understood that the degree of modification produced is not dependent solely upon the degree of dilution of the reagent. Thus smaller proportions of the 80 more concentrated mixture will produce results equivalent to those obtained with a larger proportion of the more dilute mixture. In fact the proportions of acetic anhydrid zinc chlorid and acetic acid may be varied 85 within wide limits according to the material treated and the degree of modification to be produced.

When the cellulose material has been saturated with the reagent, the action may 90 be accelerated by packing the material in a closed vessel which is placed in a thermostat regulated at a temperature of 35°-40° C. After a period of 36-48 hours at this temperature, or a longer period if the material has been left at the ordinary temperature, the reaction is complete and the cellulose is removed and washed with water until 95 free from soluble products.

When it is desirable to prevent shrinkage 100 the hanks of yarn or the fabric may be kept under tension during the treatment and during the washing also or during the washing only, if necessary.

When the cellulose is to be converted into 105 a hard, nearly waterproof material, corresponding with a gain in weight of 40-50 per cent., it should be treated with 3-4 times its weight of the more concentrated mixture, or with a smaller proportion of a 110 mixture containing less acetic acid. In the former case the cellulose should be turned over from time to time during the progress of the reaction in order that the excess of liquid may be uniformly absorbed.

Having thus described the nature of our 115 said invention and the best means we know of carrying the same into practical effect, we claim:

1. As a new article of manufacture, lower 120 acetylated derivatives of cellulose, insoluble in chloroform or nitrobenzene, made from fibrous cellulose, such derivatives having the characteristics of the original fibers that adapt the fibers for textile purposes and 125 being distinguished by resisting direct cotton dyestuffs and the action of mercerizing treatment.

2. In the process of making fibrous lower 130 acetylated derivatives of cellulose from cel-

- lulose fibers, the step which consists in treating fibrous cellulose with an appropriate acetylating agent until there is an increase in its weight not exceeding 50 per cent. without appreciable alteration of the textile qualities of the fiber, substantially as described.
3. In the process of making fibrous lower acetylated derivatives of cellulose fibers, the 10 step which consists in subjecting the fibrous cellulose to the action of a mixture of acetic anhydrid and a saline condensing agent that has no appreciable injurious effect on the fiber, such as zinc chlorid, and continuing such action until there is an increase in the weight of the cellulose not exceeding 50 per cent., without appreciable alteration of the textile qualities of the fiber, substantially as described.
- 15 4. In the process of making fibrous lower acetylated derivatives of cellulose from cellulose fibers, first saturating the cellulose with a mixture of acetic anhydrid and zinc.

chlorid suitably diluted with glacial acetic acid, then heating the saturated cellulose in a closed vessel at a temperature of 35-40° C. for some hours until the cellulose is converted into lower acetyl derivatives without appreciable alteration of the textile qualities of the fiber, and finally washing and drying the material.

5. In the process of making an acetylating agent for the purpose herein defined, introducing acetyl chlorid and a zinc compound capable of reacting therewith to form zinc chlorid, into a mixture containing acetic anhydrid and glacial acetic acid.

In testimony whereof we have signed our names to this specification in the presence of two subscribing witnesses.

CHARLES FREDERICK CROSS.  
JOHN FREDERICK BRIGGS.

Witnesses:

JOSEPH WILLARD,  
T. J. OSMAN.